

## UNITED STATES PATENT OFFICE.

CHARLES FRANK SAMMET, OF DALTON, MASSACHUSETTS, ASSIGNOR TO CRANE & COMPANY, OF DALTON, MASSACHUSETTS, A PARTNERSHIP.

## SAFETY PAPER AND PROCESS OF MAKING THE SAME.

No Drawing.

Application filed October 31, 1921. Serial No. 511,808.

To all whom it may concern:

Be it known that I, CHARLES FRANK SAMMET, a citizen of the United States, residing at Dalton, in the county of Berkshire, State of Massachusetts, have invented certain new and useful Improvements in Safety Paper and Processes of Making the Same, of which the following is a description.

10 My invention relates to an improved process for the manufacture of safety paper for checks, notes, bonds, wills and other documents, and has for its object the production of a paper of such character that 15 any attempt to obliterate or remove writing, printing or other marks thereon by chemical means will cause a marked change in the appearance or color of the paper where the chemical has been brought in contact with 20 the surface, as a result of which changes in the writing or printing or other marks will be more apparent and the fraud easily detected.

It will also be understood that the invention 25 is applicable either to plain white or tinted paper, as well as to paper having surface markings thereon for the purpose of indicating when mechanical erasures of the writing or marking thereon have been 30 made.

In the manufacture of this safety paper by incorporation of the ingredients applied thereto in the body of the paper, I make use of any of the usual well-known processes 35 for the manufacture of paper, and the material to be used in the process for making the safety paper and for the purpose of accomplishing the result, is incorporated in the paper at any desirable stage of the manufacture—either while the paper is in the pulp stage; on the web; or the material may be added during the sizing operation.

The essential feature of the invention consists in the incorporation therewith at any 45 desirable stage in the manufacture of the paper of a member of the benzidine group, such as benzidine or its homologues, substitution products, derivatives or salts. Of this I prefer benzidine, ortho-tolidin and ortho-dianisidine, and I find the most useful to be an insoluble salt of benzidine and of these I prefer the sulphate.

While, as above stated, the safety material 55 may be incorporated with the paper at any suitable stage in its manufacture—that is, in

the pulp, in the web, after or with the sizing—it will also be understood that it may be applied as a coating to the otherwise finished paper; or, when desired, it may be applied by incorporating it with the ink used for marking the paper. I also consider the invention broad enough to include the application of the safety material to the finished paper either in the form of a powder or suspended in a liquid or as a solution. In fact, in a co-pending application Serial No. 511,510, executed of even date herewith, I have set forth a way of applying the material to the finished paper by molding the material in the form of sticks somewhat analogous in size and shape of the well known sticks of shaving soap, the molding being accomplished under pressure or by incorporating a small amount of binder, such as starch, with the material sufficient to hold the particles together. This stick may be rubbed over the paper manually with the exertion of slight pressure and the excess material may then be removed either by blowing or dusting it off. A sufficient amount will remain incorporated in the surface of the paper to produce the desired result.

When the paper is manufactured by incorporation of the safety material during the process of manufacture of such paper, I have found substantially the following proportions give the best results, viz: 100 parts by weight of pulp to 5 parts of the benzidine salt, although it will be understood that these proportions may be varied without departing from the spirit of the invention.

The substances of the class named, and especially those substances mentioned, are discolored upon treatment with ink eradicators, which usually contain oxidizing agents, the change being due to the oxidizing effect of the eradicator, although other ingredients thereof may also produce a color change in the safety material. A dirty brown spot is usually produced upon the paper with which they are in contact, which spot cannot be obliterated by treatment with acids, alkalis, reducing agents or other chemicals.

I have found that the safety substances I propose to use are best used in the form of insoluble salts, for example, as sulphates, since the color of the benzidine or other sulphate or other insoluble salts are practically unaffected by long exposure to light, while

the soluble salts are somewhat darkened by long exposure thereto.

The stain produced by treatment with an oxidizing agent cannot be removed by treatment with acids or alkalis or reducing agents; however, should a reducing agent be present during the treatment with an oxidizing agent the stain may not appear until the reducing agent has been oxidized.

10 I use the variety of tolidin and dianisidine sold as such upon the market and believe these to have the ortho-structure.

In a co-pending application Serial No. 511,809, designated as Case II, I have 15 claimed the process of making safety paper and the product itself having diphenylamin incorporated therewith, and the application heretofore referred to as relating to the stick of safety material is designated as

20 Case III, Serial No. 511,810.

Having thus described my invention, what I claim as new and desire to secure by Letters Patent, is:

1. The process of making safety paper 25 which consists in adding to the paper a material which is a colorless member of the benzidine group or its homologues.

2. The process of making safety paper which consists in adding to the paper a salt 30 of the benzidine group or homologues thereof.

3. The process of making safety paper which consists in adding to the paper an insoluble salt of benzidine.

35 4. The process of making safety paper which consists in adding to the paper benzidine sulphate.

5. The process of making safety paper 40 which consists in adding to the paper benzidine sulphate in substantially the following proportions—100 parts by weight of pulp to 5 parts by weight of benzidine salt.

6. Paper, having a colorless member of the benzidine group incorporated therewith.

45 7. Paper, having a colorless member of the benzidine group incorporated therein.

8. Paper, having a salt of a member of the benzidine group incorporated therewith.

9. Paper, having a salt of a member of the benzidine group incorporated therein. 50

10. Paper, having an insoluble salt of a member of the benzidine group incorporated therewith.

11. Paper, having an insoluble salt of a member of the benzidine group incorporated 55 therein.

12. Paper, having an insoluble compound of a member of the benzidine group incorporated therewith.

13. Paper, having an insoluble compound 60 of a member of the benzidine group incorporated therein.

14. Paper, having a sulphate of a member of the benzidine group incorporated therewith. 65

15. Paper, having a sulphate of a member of the benzidine group incorporated therein.

16. Paper, having benzidine incorporated 70 therein.

17. Paper, having benzidine incorporated therein.

18. Paper, having a salt of benzidine incorporated therewith.

19. Paper, having a salt of benzidine incorporated therein. 75

20. Paper, having an insoluble compound of benzidine incorporated therewith.

21. Paper, having an insoluble compound of benzidine incorporated therein. 80

22. Paper, having an insoluble salt of benzidine incorporated therewith.

23. Paper, having an insoluble salt of benzidine incorporated therein.

24. Paper, having benzidine sulphate incorporated therewith. 85

25. Paper, having benzidine sulphate incorporated therein.

In testimony whereof, I affix my signature.

CHARLES FRANK SAMMET.